# EUROPEAN PATENT SPECIFICATION

(11) **EP 0 044 381 B1**
(45) Date of publication and mention of the grant of the patent: **03.04.1985**
(21) Application number: 81103570.8
(22) Date of filing: 11.05.1981
(51) Int. Cl.: G21F 9/36

(54) **Method for treating radioactive material and container for enclosing such material**
Verfahren zur Behandlung radioaktiven Materials und Behälter zur Lagerung solchen Materials
Méthode pour traiter les matériaux radioactifs et récipient pour enfermer de tels matériaux

(30) Priority: 19.05.1980 SE 8003699; 19.05.1980 SE 8003698
(43) Date of publication of application: 27.01.1982
(73) Proprietor: ASEA AB, S-721 83 Västeras (SE)
(72) Inventor: Larker, Hans, S-915 00 Robertsfors (SE); Tegman, Ragnar, S-902 37 Umeä (SE)
(74) Representative: Boecker, Joachim, Dr.-Ing.

## Description

The invention relates to a method of treating material including radioactive material according to the prior art portion of claim 1 and a container used in said method.

During reprocessing of nuclear fuel, separated high-level waste material must be treated and stored so as to prevent spreading into the biosphere. The first stage is to transform the waste into solid state and, for example, convert it into a solid, crystalline material having good chemical resistance and being capable of resisting leaching by water. One way of achieving this is to compress, at a high temperature and a high pressure, a mixture of waste and a resistant material in particulate form into a massive, solid body where the active material becomes permanently bound. A method of achieving such a solid body is disclosed in US Patent 4,172,807. Radioactive metal scrap or radioactive ashes may be treated in a similar manner.

A problem when transforming the waste into solid state is the contamination of the equipment used in the process. In the method according to the above-mentioned patent, containers may be filled with waste material in particulate form and sealed in a relatively simple manner. The equipment used for the filling and the sealing is relatively simple and may therefore be cleaned in a simple manner prior to any necessary repair work. The furnace equipment for the hot pressing, on the other hand, is complicated and much more difficult to clean after a possible contamination.

From the US-A-3 160 502 it is known, to compress beryllium powder or beryllium chips into a solid body with the help of a hydraulic press. The beryllium powder or the beryllium chips are filled in an evacuated and sealed container which has a bellows-shaped side wall. During the compression the top and bottom end of the container are firmly gripped between the two pressure applying plates of the hydraulic press. This firm grip prevents the top and bottom end from bending laterally. The danger of distortion of the container is therefore virtually eliminated. Furthermore, the pressure on the container is applied at very high speed so that the compression of the container takes place almost instantaneously.

Compressing material of the afore-mentioned type in a bellows-shaped container with a hydraulic press carries the disadvantage that a compression to theoretical density is unachiev- able and that the density of the compressed material is not homogeneous. Particularly the material trapped in the crevices formed by the compressed corrugated side walls of the container shows a very low density. This is particularly harmful with radioactive material, which is prone to leaching if the density is unsufficient. Furthermore the method known from US-A-3 160 502 is not usable for a material, which has a very low fill factor like particulate or piece-formed material.

The invention aims at further developing a method of the above-mentioned kind which allows to compress material including radioactive particulate or piece-formed material to a solid body of extremely high and homogeneous density.

In order to achieve this aim the invention suggests a method of the above-mentioned kind, which is characterised by the features of the characterising portion of claim 1.

Further developments of the method according to the invention are characterised by the features of the claims 2 to 5.

A container usable in the method according to the invention is characterised by the features of claim 6. Further developments of such a container carry the features of the claims 7 to 10.

By hot isostatic pressing the material in the container is transformed into a solid body of extremely high and homogeneous density.

The invention thus relates, on the one hand, to a method of enclosing radioactive particulate or piece-formed material in a redundant gas-tight container and converting the material into a solid body by compression at a necessary high temperature and a necessary high pressure in an isostatic press, and on the other hand to a container for enclosing the above-mentioned material. The material to be contained may consist of a mixture of radioactive material and a material resistant to leaching by water. A risk of contamination of the furnace and its gas supply system may arise if pressure gas should leak into the capsule during the pressing and, during the decompression after the pressing, blow out radioactive material from the container. The container is suitably made as a multi-layer container to make it redundant, thus in all essentials eliminating the risk of leakage. The container is built up of two or more capsules, arranged one inside the other, of different materials, for example of titanium and stainless steel. When the material to be contained possesses such properties that it cannot be packed into high density when filling the container, problems will often occur during the pressing because of great distortion during the compression. A long capsule may be bent to such an extent that it will get into contact with the walls of the furnace space or with heating elements in the furnace, resulting in the furnace being damaged and in difficulties in removing the pressed container. Distortion problems arise at a fill factor of about 60% and are accentuated with decreasing fill factor. The difficulties in achieving such a high fill factor as 60% are especially great when it is a question of enclosing pieces of cladding tubes.

According to the invention, the distortion problems are reduced and the compression is facilitated by enclosing the material to be compressed in a container of such a shape that an axial compression of the container is facilitated. The container may be made with a corrugated sheath with a substantially plane lid and plane bottom, or with a cylindrical sheath with a lid and/or bottom which is/are joined to the sheath by a bellows projecting into the sheath. This bellows or these bellows make possible an axial insertion of the lid and the bottom and an axial compression of the contained material. Also containers with a cylindrical side wall and a corrugated lid and bottom can be used. The material contained in the container is according to the invention converted into a solid body by isostatic compression at a high temperature.

The filling density may be increased prior to the hot pressing by an axial compression of the container in cold condition. When enclosing tubular pieces of cladding material, which may have as low a fill factor as 10-15%, this precompac- tion prior to the hot pressing is particularly desirable. This compression may be carried out between press tables or between pistons in a hydraulic press or isostatically in a pressure chamber under the influence of a gaseous or liquid pressure medium. This latter method of pressing is possible for a container with a corrugated sheath side wall because of its great radial stiffness but small axial stiffness. The compression before the hot pressing to a density exceeding 70% of the theoretical density is desirable. The axial compression of the material in the capsule results in a smaller radial compression of the sheath during the final hot pressing into a solid body than what would otherwise be the case. This contributes effectively to reduce the distortion during the hot pressing. During the compression before the hot pressing the container is suitably placed in a container with axial guide means preventing bending of the container during its axial compression.

The corrugated sheath and the bellows also facilitate the axial compression during the hot pressing. During the pressing in the pressure furnace a somewhat greater axial compression is obtained than with a container of a conventional design.

The invention will be described in greater detail with reference to the accompanying drawing, in which:
Figure 1 shows an example of a container according to the invention with a corrugated sheath,
-Figure 2 shows another example of such a container with a smooth sheath and with a lid and a bottom which are joined to the sheath by bellows,
Figures 3 and 4 show further embodiments of containers according to the invention with a corrugated lid and bottom.

The container 1 according to Figure 1 is constructed with a corrugated sheath 2, with a plane bottom 3 and with a plane lid 4. The opening of the lid 4 is gas-tightly sealed by the lid 5. The container 1 is built up of two sheet-metal capsules arranged one inside the other, the sheaths, bottom and lids of said capsules being designated 2a, 2b, 3a, 3b, 4a, 4b and 5a, 5b. The container 1 is filled with a radioactive material 6. The material in the inner capsule may be titanium, and in the outer capsule stainless steel.

The container 11 according to Figure 2 is constructed with a cylindrical sheath 12, a plane bottom 13 which is joined to the sheath 12-by a bellows 14, projecting into the container 11, and a lid 15 which is joined to the sheath 12 by a bellows 16 projecting into the container 11. The opening of the lid 15 is sealed by a lid 17. The container 11 is built up of two sheet-metal capsules arranged one inside the other, the sheaths, bottoms, bellows and lids of which are designated 12a, 12b, 13a, 13b, 14a, 14b, 16a, 16b, 15a and 15b. The container 11 is filled with a radioactive material 6.

The container 19 of Figure 3 is composed of two bottle-shaped capsules 20 and 21. The inner capsule 20 may consist of, for example, titanium, the outer of, for example, stainless steel. The inner capsule 20 is made with a relatively small neck 22 with a flange 23 and is sealed by a lid 24 which, after the filling, is gas-tightly joined to the flange 23 by welding. The capsule 21 is formed with an opening 25 with an inclined flange 26. A lid composed of parts 27 and 28 is adapted to the opening 25. Part 27 of this lid is formed with a flange 29 which, when sealing the capsule 21, is gas-tightly joined to the flange 26 by welding. The space between the neck 22 and the lid 27, 28 is filled with a supporting metal block 30, which prevents too great a deformation of the lid part 27 during the pressing. The bottom portions of the capsule parts 20 and 21 as well as their upper end portions are constructed with annular corrugations 31, 32 and 33, 34, respectively. These facilitate an axial compression of the capsule during the initial stage of the pressing and provide a certain axial compaction which eliminates, or at least reduces, the distortion of the capsule during the pressing. The capsule is supported on a supporting ring 36.

Figure 4 shows the container according to Figure 3 after the pressing. The contents 35, for example scrap of cladding tubes, have been pressed to practically full density.

Containers of the kind described above may have a length of between 2000 and 3000 mm and a diameter of 500-600 mm. The capsules 20 and 21 and their respective lids are bonded together after the pressing.

## Claims

1. Method of treating material including radioactive particulate or piece-formed material (6) by enclosing the material in a gastight container (1) having at least one corrugated or bellows-like wall portion (2, 14, 16, 31, 32, 33, 34) and compressing the material (6) into a solid body at a necessary temperature and a necessary pressure, characterised in that the conversion of the material (6) into a solid body takes place by isostatic pressing at a high temperature and in that the container is substantially unsupported against lateral bending.

2. Method according to claim 1, characterised in that the containers (1, 11) after filling of the material (6) is compressed axially at room temperature prior to the final high temperature isostatic pressing.

3. Method according to claim 2, characterised in that the compression is carried out so that the material (6) in the containers (1, 11) is densified to 40% or more of the theoretically possible density.

4. Method according to claim 2 or 3, characterised in that the compression at room temperature is carried out mechanically.

5. Method according to claim 2 or 3, characterised in that the compression at room temperature is carried out isostatically in a pressure chamber under the influence of a gaseous or liquid pressure medium.

6. Container (1, 11, 19) used in the method according to any of the preceding claims for enclosing material including radioactive particulate or piece-formed material (6, 35) which is converted into a solid body by isostatic pressing at a high temperature, characterised in that the walls of said container are provided with at least one corrugated wall portion (2, 14, 16, 31, 32, 33, 34).

7. Container according to claim 6, characterised in that said wall portion consists of a bellows-like side wall (2; Figure 1).

8. Container according to claim 6, characterised in that said container (11) has a cylindrical sheath (12) with a lid (15) and/or a bottom (13) which are joined to the sheath (12) by said wall portion which consists of bellows (14, 16) projecting into said cylindrical sheath (12; Figure 2).

9. Container according to claim 6, characterised in that said container (11) has a cylindrical sheath with a lid and a bottom and that said wall portion consists of a bottom and/or lid portion provided with annular corrugations (31, 32, 33, 34; Figure 3).

10. Container according to any of claim 6 to 9, characterised in that the container (1, 11, 19) is built up from at least two capsules (2a, 2b, 12a, 12b, 20, 21), one within the other.

## Revendications

1. Procédé de traitement d'une matière comprenant de la matière (6) radioactive en particules ou en morceaux, en enfermant la matière dans un récipient (1) étanche aux gaz ayant au moins une portion de paroi (2, 14, 16, 31, 32, 33, 34) ondulée ou semblable à un soufflet, et en comprimant la matière (6) en un corps solidé à une température et sous la pression qui sont nécessaires, caractérisé en ce qu'il consiste à effectuer la transformation de la matière (6) en un corps solide, par compression isostatique à une température élevée, et en ce que le récipient n'est pratiquement pas supporté en vue d'être protégé d'un flambage latéral.

2. Procédé suivant la revendication 1, caractérisé en ce qu'il consiste à comprimer axialement les récipients (1, 11) à la température ambiante, après les avoir emplis de la matière (6) et avant la compression isostatique finale à température élevée.

3. Procédé suivant la revendication 2, caractérisé en ce qu'il consiste à effectuer la compression de manière à densifier la matière (6) dans les récipients (1,11), jusqu'à 40% ou davantage de la masse volumique qui est possible théoriquement.

4. Procédé suivant la revendication 2 ou 3, caractérisé en ce qu'il consiste à effectuer la compression à température ambiante par voie mécanique.

5. Procédé suivant la revendication 2 ou 3, caractérisé en ce qu'il consiste à effectuer la compression à la température ambiante par voie isostatique dans une chambre de pression, sous l'influence d'un milieu de pression gazeux ou liquide.

6. Récipient (1, 11, 19) utilisé dans le procédé suivant l'une des revendications précédentes, pour enfermer de la matière comprenant de la matière (6, 35) radioactive en particules ou en morceaux, qui est transformée en un corps solide par compression isostatique à une température élevée, caractérisé en ce que les parois du récipient sont munies d'au moins une portion de paroi ondulée (2, 14, 16, 31, 32, 33, 34).

7. Récipient suivant la revendication 6, caractérisé en ce que la portion de paroi consiste en une portion de paroi semblable à des soufflets (27; figure 1).

8. Récipient suivant la revendication 6, caractérisé en ce que le récipient (11) a une enveloppe (12) cylindrique, avec un couvercle (15) et/ou un fond (13) qui sont réunis à l'enveloppe (12) par la portion de paroi, qui consiste en soufflets (14, 16) faisant saillie dans l'enveloppe cylindrique (12; figure 2).

9. Récipient suivant la revendication 6, caractérisé en ce que le récipient (11) a une enveloppe cylindrique avec un couvercle et un fond et la portion de paroi consiste en une portion de fond et/ou de couvercle munis d'ondulations annulaires (31, 32, 33, 34; figure 3).

10. Récipient suivant l'une des revendications 6 à 9, caractérisé en ce que le récipient (1, 11, 19) est constitué d'au moins deux capsules (2a, 2b, 12a, 12b, 20, 21) l'une dans l'autre.

## Patentansprüche

1. Verfahren zur Behandlung von Material, welches partikelförmiges oder stückförmiges radioaktives Material (6) enthält, bei welchem Verfahren das Material in einem gasdichten Behälter (1) eingeschlossen wird, welcher zumindest einen gewellten oder faltenbalgartigen Wandabschnitt (2, 14, 16, 31, 32, 33, 34) hat, und bei welchem Verfahren das Material (6) bei einer erforderlichen Temperatur und einem erforderlichen Druck zu einem festen Körper gepreßt wird, dadurch gekennzeichnet, daß die Umwandlung des Materials (6) in einen festen Körper durch isostatisches Pressen bei hoher Temperatur erfolgt und daß der Behälter im wesentlichen nicht gegen seitliches Biegen abgestützt ist.

2. Verfahren nach Anspruch 1, dadurch gekennzeichnet, daß die Behälter (1, 11) nach dem Einfüllen des Materials (6) bei Raumtemperatur in axialer Richtung komprimiert werden, bevor das, abschließende isostatische Pressen bei hoher Temperatur erfolgt.

3. Verfahren nach Anspruch 2, dadurch gekennzeichnet, daß die Kompression in der Weise ausgeführt wird, daß das Material (6) in den Behältern (1, 11) auf 40 Prozent oder mehr der theoretisch möglichen Dichte verdichtet wird.

4. Verfahren nach einem der Ansprüche 2 oder 3, dadurch gekennzeichnet, daß die bei Raumtemperatur erfolgende Kompression mechanisch erfolgt.

5. Verfahren nach einem der Ansprüche 2 oder 3, dadurch gekennzeichnet, daß die bei Raumtemperatur erfolgende Kompression isostatisch in einer Druckkammer mittels eines gasförmigen oder flüssigen Druckmittels erfolgt.

6. Behälter (1, 11, 19) zur Verwendung bei dem Verfahren gemäß einem der vorhergehenden Ansprüche zum Einschließen von Material, welches partikelförmiges oder stückförmiges radioaktives Material (6, 35) enthält und welches durch isostatisches Pressen bei hoher Temperatur in einen festen Körper umgewandelt wird, dadurch gekennzeichnet, daß die Wände des genannten Behälters mindestens einen wellenförmigen Wandabschnitt (2, 14, 16, 31, 32, 33, 34) haben.

7. Behälter nach Anspruch 6, dadurch gekennzeichnet, daß der genannte Wandabschnitt aus einer faltenbalgartigen Seitenwand (2) besteht (Figur 1).

8. Behälter nach Anspruch 6, dadurch gekennzeichnet, daß der genannte Behälter (11) aus einer zylindrischen Hülle (12) mit einem Deckel (15) und/oder einem Boden (13) aufgebaut ist, der/die mit der Hülle (12) über einen der genannten faltenbalgartigen Wandabschnitte (14, 16), welcher in die zylindrische Hülle (12) hineinragt, verbunden ist/sind (Figur 2).

9. Behälter nach Anspruch 6, dadurch gekennzeichnet, daß der genannte Behälter (11) eine zylindrische Hülle mit einem Deckel und einem Boden umfaßt und daß der genannte Wandabschnitt aus einem Boden- und/oder Deckelabschnitt besteht, der/die mit einer ringförmigen Wellung (31, 32, 33, 34) versehen ist/sind (Figur 3).

10. Behälter nach einem der Ansprüche 6 bis 9, dadurch gekennzeichnet, daß der Behälter (1, 11, 19) aus mindestens zwei Kapseln (2a, 2b, 12a, 12b, 20, 21) aufgebaut ist, von denen die eine in der anderen angeordnet ist.
